# EUROPEAN PATENT APPLICATION

(11) **EP 4 733 458 A1**
(43) Date of publication of application: **29.04.2026**
(21) Application number: 24825690.1
(22) Date of filing: 31.05.2024
(51) Int. Cl.: D04B 1/00, A41B 9/00, A41D 31/00, A41D 31/06, D02G 3/04, D04B 1/14

(54) **KNITTED FABRIC AND CLOTHING CONTAINING THE SAME**

(30) Priority: 23.06.2023 JP 2023103065
(71) Applicant: Toray Industries, Inc., Tokyo 103-8666 (JP)
(72) Inventor: ABE, Wataru, Tokyo 103-8666 (JP); NARUKO, Satoshi, Osaka-shi, Osaka 530-8222 (JP)
(74) Representative: Mewburn Ellis LLP
(86) International application number: PCT/JP2024/020016
(87) International publication number: WO 2024/262283

(57) **Abstract**

The present invention is to provide a knitted fabric excellent in skin surface smoothness, heat retaining property, and wash and wear property, and an excellent clothing including the knitted fabric, and relates to a knitted fabric having a single knit structure, wherein a course of a fiber 1 made of a spun yarn and a course of a fiber 2 made of a long fiber are alternately and repeatedly present in a warp direction, a ratio (D2/D1) of a total fineness D2 of the fiber 2 to a total fineness D1 of the fiber 1 is in a range of 0.50 to 0.90, and a ratio (L2/L1) of a yarn length L2 of the fiber 2 to a yarn length L1 of the fiber 1 per 100 wales is greater than 1.00.

## Description

### TECHNICAL FIELD

The present invention relates to a knitted fabric and a clothing.

### BACKGROUND ART

Conventionally, attempts have been made to combine the heat retaining property imparted by spun yarn with the wash and wear property imparted by long fibers in heat-retaining fiber products for innerwear applications. For example, a knitted fabric including a viscose rayon fiber, a cation-dyeable polyester fiber, a polyacrylic synthetic fiber, and a polyurethane-based elastic fiber is known (see, for example, Patent Document 1 and Patent Document 2).

In addition, an attempt to improve the heat retaining property by including dead air in the knitted fabric through forming an interlock structure and adopting a specific loop balance in order to improve the heat retaining property is also known (see, for example, Patent Document 3).

### PRIOR ART DOCUMENTS

### PATENT DOCUMENTS

Patent Document 1: Japanese Patent No. 6,447,128
Patent Document 2: Japanese Patent No. 5,453,863
Patent Document 3: Japanese Patent No. 6,635,972

### SUMMARY OF THE INVENTION

### PROBLEMS TO BE SOLVED BY THE INVENTION

In consideration of heat retaining property in clothing, it is preferable to apply a method using a spun yarn and a long fiber as described in Patent Documents 1 and 2, or to provide bulkiness by an interlock structure or the like as described in Patent Document 3.

On the other hand, for example, in undergarments and the like, a thin, soft, and smooth knitted fabric is preferred. However, according to findings by the present inventors, a thin and soft single knit structure has an uneven skin surface, and thus has a problem of touch feeling. Furthermore, for example, when a spun yarn and a long fiber are used for the wash and wear property in addition to improving the heat retaining property as described in Patent Document 1 and Patent Document 2, the spun yarn is thick and the long fiber is thin, and thus, the unevenness of a single knit fabric becomes more remarkable.

In addition, the technique of Patent Document 3 is excellent in heat retaining property and does not cause a problem of surface smoothness, but causes a problem of thickness and flexibility.

Therefore, an object of the present invention is to provide a knitted fabric that is thin and soft and is also excellent in skin surface smoothness, heat retaining property, and wash and wear property, and a clothing including the knitted fabric.

### SOLUTIONS TO THE PROBLEMS

In order to solve the problems described above, the present invention has the following configuration.
(1) A knitted fabric having a single knit structure, wherein a course of a fiber 1 made of a spun yarn and a course of a fiber 2 made of a long fiber are alternately present in a warp direction, a ratio (D2/D1) of a total fineness D2 of the fiber 2 to a total fineness D1 of the fiber 1 is in a range of 0.50 to 0.90, and a ratio (L2/L1) of a yarn length L2 of the fiber 2 to a yarn length L1 of the fiber 1 per 100 wales is greater than 1.00.
(2) The knitted fabric according to (1), wherein the spun yarn contains a cellulose fiber and an acrylic fiber.
(3) The knitted fabric according to (1) or (2), wherein a total fineness of the fiber 1 is 70 decitex to 150 decitex.
(4) The knitted fabric according to any one of (1) to (3), wherein the long fiber is a cation-dyeable polyester long fiber.
(5) The knitted fabric according to any one of (1) to (4), wherein the total fineness of the fiber 2 is 33 decitex to 135 decitex.
(6) The knitted fabric according to any one of (1) to (5) further including an elastic fiber.
(7) The knitted fabric according to any one of (1) to (6) further including a course of an elastic fiber.
(8) The knitted fabric according to any one of (1) to (7), wherein the ratio (L2/L1) of the yarn length L2 of the fiber 2 to the yarn length L1 of the fiber 1 per 100 wales is in a range of 1.02 to 1.20.
(9) A clothing including the knitted fabric according to any one of (1) to (8).
(10) An undergarment or underwear made of the knitted fabric according to any one of (1) to (8).

### EFFECTS OF THE INVENTION

According to the present invention, a knitted fabric excellent in skin surface smoothness, heat retaining property, and wash and wear property, and a clothing including the knitted fabric can be obtained.

### BRIEF DESCRIPTION OF THE DRAWINGS

Fig. 1 is a schematic view of a knitted fabric illustrating one embodiment of the present invention.

### EMBODIMENTS OF THE INVENTION

An embodiment of a knitted fabric of the present invention will be described in detail. The knitted fabric of the present invention includes a course of a fiber 1 made of a spun yarn and a course of a fiber 2 made of a long fiber. A heat retaining property can be improved by the spun yarn. In addition, the long fiber is excellent in wash and wear property, and in the present invention, the strength and wrinkle resistance of a single knit fabric can be improved. Fibers other than spun yarn may be included in the fiber 1, and fibers other than long fibers may be included in the fiber 2, insofar as they do not hinder the effects of the present invention.

In the present invention, the spun yarn is not particularly limited, and one or a plurality of types of natural fibers such as cotton, hemp, and wool, chemical fibers such as rayon and acetate, and synthetic fibers such as polyester, acrylic, and nylon may be used. In the present invention, it is preferable that the spun yarn contains cellulose fiber such as cotton, rayon, and acetate and acrylic fiber from the viewpoint of heat retaining property.

The cellulose fiber is not particularly limited, but is preferably a viscose rayon fiber. The viscose rayon fiber is a regenerated fiber which is spun by a viscose method and is a short fiber such as a viscose rayon fiber or a saponified acetate fiber. It is preferable that the mass fraction of the cellulose fiber to the spun yarn is 15 mass% or more. When the cellulose fiber is contained in the above range, a knitted fabric having excellent durability and moisture-induced exothermicity can be obtained. Since the knitted fabric has moisture-induced exothermicity, etc., the knitted fabric generates heat by water vapor emitted from a human body when worn, and the temperature of a garment can be increased. The mass fraction of the cellulose fiber to the spun yarn is preferably 60 mass% or less, and more preferably 40 mass% or less. By setting the upper limit of the cellulose fiber within the above range, wrinkles can be further suppressed after washing.

The acrylic fiber is not particularly limited, and may be a regular type polyacrylic fiber made of polyacrylonitrile, an acrylic fiber obtained by copolymerizing or adding another compound based on an acrylic composition, or a polyacrylic fiber modified to an anti-pilling type, a water-absorbing type, etc. The mass fraction of the acrylic fiber to the spun yarn is preferably 40 mass% or more, and more preferably 60 mass% or more. When the acrylic fiber is contained in the above range, an effect of further improving the heat retaining property is exhibited. The mass fraction of the acrylic fiber to the spun yarn is preferably 80 mass% or less, and more preferably 70 mass% or less. By setting the upper limit of the content ratio of the acrylic fiber within the above range, the content ratio of, for example, the cellulose fiber can be relatively improved, and the moisture-induced exothermicity can be improved.

It is preferable that the single fiber fineness of the acrylic fiber is 0.6 decitex or more from the viewpoint of softer texture, improvement in heat retaining property, improvement in spinning property, strength, etc. From the viewpoint of texture, the single fiber fineness of the acrylic fiber is preferably 2.2 decitex or less, and more preferably 1.5 decitex or less.

Considering that the knitted fabric of the present invention can be used preferably for undergarments, T-shirts, and the like that directly contact human skin, the total fineness of the fiber 1 is preferably 150 decitex or less, and more preferably 130 decitex or less from the viewpoint of excellent touch feeling and flexibility. In addition, from the viewpoint of excellent heat retaining property, the total fineness of the fiber 1 is preferably 70 decitex or more, and more preferably 90 decitex or more. It is preferable that the single fiber fineness of the spun yarn is 0.5 decitex to 2.5 decitex from the viewpoint of usage. It is preferable that the spun yarn is composed of short fiber, and the fiber length of the spun yarn is in a range of 38 mm to 52 mm.

In the present invention, the long fiber is not particularly limited, and for example, monofilaments and multifilaments made of chemical fiber such as rayon and acetate and synthetic fiber such as polyester, nylon, and acrylic can be appropriately used. Among them, polyester long fiber is preferable from the viewpoint of strength and wrinkle resistance. Examples of polyester long fiber include polyethylene terephthalate long fiber, polybutylene terephthalate long fiber, polytrimethylene terephthalate long fiber, and long fiber of copolymers thereof, and in addition to single component long fiber, composite long fiber having a cross section such as side-by-side and core-sheath can also be used. In the present invention, in consideration of dyeability with other materials, for example, a cation-dyeable polyester long fiber that can be dyed with a cationic dye, such as a polyethylene terephthalate long fiber copolymerized with 1.0 mol% to 3.0 mol% of a 5-sodium sulfoisophthalic acid component, is preferable. By using the cation-dyeable polyester long fiber, it is possible to perform dyeing at a lower temperature than that of a normal polyester fiber, and it is also possible to perform dyeing with the same dye as the acrylic fiber. In addition, since the cation-dyeable polyester long fiber can obtain excellent color developability and fastness at a temperature of 105°C to 115°C, it is possible to suppress deterioration due to heat of other fibers, particularly when a polyurethane-based elastic fiber is contained.

In the production of the cation-dyeable polyester long fiber, a method of producing polyester which is generally known can be used. In addition, as is generally known, cationic dyeability of a normal polyester is achieved by, for example, copolymerizing the normal polyester with 1.0 mol% to 3.0 mol% of a 5-sodium sulfoisophthalic acid component.

In the present invention, the fiber 2 is preferably a multifilament, and at this time, the number of filaments is preferably 24 to 192. The total fineness of the fiber 2 is preferably 135 decitex or less, more preferably 120 decitex or less, and still more preferably 100 decitex or less from the viewpoint of excellent touch feeling and flexibility considering that the knitted fabric of the present invention can be preferably used for undergarments, T-shirts, and the like that directly contact human skin. In addition, in terms of excellent strength, the total fineness of the fiber 2 is preferably 33 decitex or more, more preferably 40 decitex or more, and still more preferably 50 decitex or more.

The mass fraction of the fiber 2 to the knitted fabric is preferably 20 mass% or more, and more preferably 30 mass% or more. Within the above range, the occurrence of wrinkles of the fiber structure body after washing can be further suppressed. The mass fraction of the fiber 2 to the knitted fabric is preferably 60 mass% or less, and more preferably 50 mass% or less. Within the above range, the heat retaining property can be improved.

In the present invention, it is preferable that the fiber 1 and the fiber 2 described above exist in separate courses.

A preferable aspect of the knitted fabric of the present invention is to further contain elastic fiber from the viewpoint of wearing comfort. More preferably, it is an aspect including a course of an elastic fiber. The elastic fiber is contained in an amount of preferably 3 mass% or more, more preferably 5 mass% or more with respect to the knitted fabric. Within the above range, it is possible to increase an appropriate elongation and a gap between knitted fabric loops, thereby exhibiting an effect of smoothly following the movement of the body and further improving the wearing comfort. In addition, the elastic fiber is contained at a ratio of preferably 15 mass% or less and more preferably 13 mass% or less with respect to the knitted fabric. Within the above range, an effect of reducing excessive tightening at the time of wearing by the elastic fiber and improving the wearing comfort is exhibited.

As the elastic fiber, a polyurethane-based elastic fiber is preferable in terms of cost and stretchability. It is preferable that the polyurethane-based elastic fiber has an elastic recovery at 200% elongation of 90% or more. Within the above range, excellent durability against repeated wearing can be obtained. In addition, a knit structure and a knit density can be arbitrarily set depending on an intended use. In addition, the total fineness is preferably in a range of 15 decitex to 50 decitex, and more preferably in a range of 20 decitex to 45 decitex since the fiber is preferably used for undergarments, T-shirts, and the like which directly contact human skin. Furthermore, polyurethane-based elastic fibers are generally used in the form of long fibers (filaments), and polyurethane-based elastic fibers having a filament count of 1 to 3 are preferably used.

Furthermore, the knitted fabric of the present invention may further contain, in addition to the above, a polyester-based fiber other than those described above, a polyester-based fiber obtained by copolymerizing a third component with polyester, a polyamide-based fiber, a regenerated cellulose fiber, a protein fiber such as wool and silk, and the like. The fibers constituting the knitted fabric are used in a form of mixed fiber, mixed yarns, mixed weaves, interlaced knitting, and the like.

In the knitted fabric of the present invention, the course of the fiber 1 and the course of the fiber 2 described above are alternately and repeatedly present in the warp direction. This makes it possible to improve the heat retaining property and the strength. An aspect in which the fibers are alternately and repeatedly present is not particularly limited, and for example, as illustrated in a knitted fabric (4) of Fig. 1, an aspect in which the fiber 1 (1) and the fiber 2 (2) are alternately repeated every stage may be adopted, or the fibers may be alternately repeated in a state of being arranged in a plurality of stages including two or more stages, respectively.

In the present invention, a ratio (D2/D1) of a total fineness D2 of the fiber 2 to a total fineness D1 of the fiber 1 is in a range of 0.50 to 0.90. Here, D1 and D2 both use decitex as a unit. In the present invention, a cotton count used as a fineness unit of the spun yarn is converted to decitex by dividing 5910 by the cotton count. A specific measurement method is as described in examples described later.

The ratio (D2/D1) of the total fineness D2 to the total fineness D1 in the knitted fabric of the present invention is 0.50 or more, preferably 0.55 or more, and more preferably 0.60 or more. The ratio (D2/D1) of the total fineness D2 to the total fineness D1 in the knitted fabric of the present invention is 0.90 or less, preferably 0.85 or less, and more preferably 0.80 or less. (D2/D1) is most preferably 0.60 or more and 0.80 or less. Within the above range, even a single knit structure is excellent in smoothness, and an excellent touch feeling can be obtained.

In the knitted fabric of the present invention, a ratio (L2/L1) of a yarn length L2 of the fiber 2 to a yarn length L1 of the fiber 1 per 100 wales is greater than 1.00. The ratio is preferably 1.02 or more, more preferably 1.05 or more, and still more preferably 1.10 or more. It is preferable that the upper limit is 1.20 or less. (L2/L1) is most preferably 1.05 or more and 1.20 or less. By setting the ratio (L2/L1) of the yarn length L2 to the yarn length L1 within the above range, even a single knit structure is excellent in smoothness, and an excellent touch feeling can be obtained.

Therefore, when (D2/D1) is in a range of 0.60 or more and 0.80 or less and (L2/L1) is in a range of 1.05 or more and 1.20 or less, the smoothness is most excellent, and an excellent touch feeling can be obtained.

In general, it is known that the thinner the fiber is, the more excellent the softness and touch feeling are. However, in the present invention, it has been found that by setting the ratio (D2/D1) of the total fineness D2 to the total fineness D1 and the ratio (L2/L1) of the yarn length L2 to the yarn length L1 respectively in the above specific ranges, the unevenness of the skin surface arranged by the fiber 1 and the fiber 2 is eliminated, and effects of extremely excellent smoothness and touch feeling are exhibited.

Next, the knitted fabric of the present invention is not particularly limited as long as it is a single knit structure. With the single knit structure, thinness and flexibility can be obtained. Tissues such as jersey and inlay are preferable from the viewpoint of smoothness and touch feeling.

The clothing of the present invention includes the knitted fabric of the present invention described above. The knitted fabric of the present invention is contained in an amount of preferably 50 mass% or more of the clothing, more preferably 80 mass% or more of the clothing. The clothing is not particularly limited as long as the clothing is to be worn on a body in addition to, for example, undergarments, outerwear such as T-shirts, blousons, slacks, and skirts, and underwear such as tights, spats, camisoles, and pants, and is preferably used for various kinds of clothing. In particular, clothing that directly contacts the skin, for example, undergarments, underwear, T-shirts, tights, spats, camisole, and the like, is preferable in that the effects of the present invention can be further exhibited. Particularly preferred are undergarments and underwear.

### EXAMPLES

Next, the knitted fabric of the present invention will be specifically described based on examples. Here, methods of evaluating each performance in the examples, etc. are as described below.

### (1) Total fineness, cotton count

The cotton count of the spun yarn was measured in accordance with JIS L1095 (2010) 9.4.1. The long fiber was measured in accordance with JIS L1013 (2010) 8.3 A method, and rounded off to the nearest integer.

### (2) Yarn length (stitch length)

The yarn was unwound from the knitted fabric obtained after processing, and the stitch length (mm) at the number of stitches of 100 wales was measured in accordance with JIS L1096 (2020) 8.8, and rounded to 2 digits after a decimal point.

### (3) Ratio of total fineness D2 of fiber 2 to total fineness D1 of fiber 1 (D2/D1)

For the spun yarn, the measurement result in the above (1) was converted into decitex and obtained. The cotton count obtained in the above (1) was converted into decitex using the following formula according to the obtained count, rounded off to the nearest integer, and the resulting value was defined as D1. D2/D1 was obtained using D1 and D2, and rounded to 2 digits after a decimal point.
· D1 = 5,910/cotton count

### (4) Ratio (L2/L1) of yarn length L2 of fiber 2 to yarn length L1 of fiber 1 per 100 wales

Calculation was performed using the result measured in the above (2) and rounded to 2 digits after a decimal point.

### (5) Smoothness (tribomaster)

The measurement was conducted with a Tribomaster TL201Ts manufactured by Trinity-Lab. Inc. as a measuring device, under the test conditions of a pressing load of 10 g, a friction speed of 50 mm/sec, and the back side of the measuring surface, with the sample stretched in all directions, in a bias direction using a simulated skin sheet to obtain a coefficient of dynamic friction.

### (6) Heat retaining property (CLO value)

The measurement was conducted in accordance with ASTM D1518-85. The heat retaining property was measured using an ASTM-type heat retaining property tester at a lab temperature of 20°C and a lab humidity of 65% RH, with the back side of the fabric facing a hot plate.

### (Example 1)

40 mass% of a viscose rayon staple (single fiber fineness: 1.4 decitex, 38 mm) and 60 mass% of a polyacrylic fiber staple (single fiber fineness: 1.0 decitex, 45 mm) were mixed by card mixing to obtain a spun yarn (fiber 1) of 125 decitex.

The spun yarn thus obtained, a cation-dyeable polyester long fiber (84 decitex - 72 filaments) (fiber 2), and a polyurethane-based elastic fiber (33 decitex - 2 filaments) were knitted into a greige fabric of a jersey structure using a single-knit knitting machine having a cylinder diameter of 76.2 cm and a gauge of 28 needles/2.54 cm. As the yarn length at the time of knitting, it was designed such that, after the following processing, the spun yarn would be measured 275.00 mm and the cation-dyeable polyester long fiber would be measured 315.00 mm, alternately repeated in the warp direction, and the polyurethane-based elastic fiber was knitted in parallel with the spun yarn and the long fiber, respectively. The knitted fabric thus knitted was 30 wt% of the polyacrylic fiber, 20 wt% of a viscose rayon fiber, 38 wt% of the cation-dyeable polyester fiber, and 12 wt% of the polyurethane-based elastic fiber.

The greige fabric thus obtained was processed by steps of heat setting (190°C, 30 seconds) - scouring (70°C) - dyeing (115°C) - drying (130°C) - heat setting (130°C).

The yarn length, smoothness, and heat retaining property of the fabric thus obtained were evaluated. The results are shown in Table 1. A knitted fabric in which balance between D2/D1 and L2/L1 was excellent and both smoothness and heat retaining property were particularly excellent was obtained.

### (Example 2)

In Example 1, the knitting and processing were carried out in the same manner as in Example 1, except that the yarn length after processing was designed to be 255.00 mm of the spun yarn and 260.00 mm of the cation-dyeable polyester long fiber, and the polyurethane-based elastic fiber was 22 decitex - 2 filaments. As a result of evaluating the obtained fabric in the same manner as in Example 1, a knitted fabric excellent in both smoothness and heat retaining property was obtained as shown in Table 1.

### (Example 3)

40 mass% of a viscose rayon staple (single fiber fineness: 1.4 decitex, 38 mm) and 60 mass% of a polyacrylic fiber staple (single fiber fineness: 1.0 decitex, 45 mm) were mixed by card mixing to obtain a spun yarn of 98 decitex.

The spun yarn thus obtained, a cation-dyeable polyester long fiber (56 decitex - 72 filaments), and a polyurethane-based elastic fiber (22 decitex - 2 filaments) were knitted into a greige fabric of a jersey structure using a single-knit knitting machine having a cylinder diameter of 76.2 cm and a gauge of 28 needles/2.54 cm. As the yarn length at the time of knitting, it was designed such that, after the following processing, the spun yarn would be measured 255.00 mm and the cation-dyeable polyester long fiber would be measured 295.00 mm, alternately repeated in the warp direction, and the polyurethane-based elastic fiber was knitted in parallel with the spun yarn and the long fiber, respectively. The knitted fabric thus knitted was 32 wt% of the polyacrylic fiber, 23 wt% of a viscose rayon fiber, 32 wt% of the cation-dyeable polyester fiber, and 13 wt% of the polyurethane-based elastic fiber.

The greige fabric thus obtained was processed by steps of heat setting (190°C, 30 seconds) - scouring (70°C) - dyeing (115°C) - drying (130°C) - heat setting (130°C).

As a result of evaluating the yarn length, smoothness, and heat retaining property in the same manner as in Example 1 described above, a knitted fabric excellent in both smoothness and heat retaining property was obtained.

### (Example 4)

In Example 3, the knitting and processing were carried out in the same manner as in Example 3, except that the yarn length after processing was designed to be 255.00 mm of the spun yarn and 268.00 mm of the cation-dyeable polyester long fiber. As a result of evaluating the obtained fabric in the same manner as in Example 1, a knitted fabric excellent in both smoothness and heat retaining property was obtained as shown in Table 1.

### (Comparative example 1)

In Example 1, the jersey structure was knitted using a cation-dyeable polyester long fiber of 110 decitex in place of the spun yarn. As the yarn length at the time of knitting, it was designed such that, after the following processing, the cation-dyeable polyester long fiber of 110 decitex would be measured 275.00 mm and the cation-dyeable polyester long fiber of 84 decitex would be measured 295.00 mm, alternately repeated in the warp direction, and the polyurethane-based elastic fiber was knitted in parallel with each long fiber, respectively. The knitted fabric was 88 wt% of the cation-dyeable polyester fiber and 12 wt% of the polyurethane-based elastic fiber.

The greige fabric thus obtained was processed by steps of heat setting (190°C, 30 seconds) - scouring (70°C) - dyeing (115°C) - drying (130°C) - heat setting (130°C).

As a result of evaluating the yarn length, smoothness, and heat retaining property in the same manner as in Example 1 described above, it was confirmed that the smoothness was excellent, but the heat retaining property was poor.

### (Comparative example 2)

30 mass% of a cotton and 70 mass% of a polyacrylic fiber staple (single fiber fineness: 1.0 decitex, 45 mm) were mixed by card mixing to obtain a spun yarn of 147 decitex (cotton count: 40s).

The spun yarn thus obtained, a cation-dyeable polyester long fiber (33 decitex - 24 filaments), and a polyurethane-based elastic fiber (22 decitex - 2 filaments) were knitted into a greige fabric of a jersey structure using a single-knit knitting machine having a cylinder diameter of 76.2 cm and a gauge of 28 needles/2.54 cm. As the yarn length at the time of knitting, it was designed such that, after the following processing, the spun yarn would be measured 265.00 mm and the cation-dyeable polyester long fiber would be measured 295.00 mm, alternately repeated in the warp direction, and the polyurethane-based elastic fiber was knitted in parallel with each long fiber, respectively. The knitted fabric was 21 wt% of the cotton, 50 wt% of the polyacrylic fiber, 17 wt% of the cation-dyeable polyester fiber, and 12 wt% of the polyurethane-based elastic fiber.

The greige fabric thus obtained was processed by steps of heat setting (190°C, 30 seconds) - scouring (70°C) - dyeing (115°C) - drying (130°C) - heat setting (130°C).

As a result of evaluating the yarn length, smoothness, and heat retaining property in the same manner as in Example 1 described above, it was confirmed that the heat retaining property was excellent, but the smoothness was poor.

### (Comparative example 3)

35 mass% of a viscose rayon staple (single fiber fineness: 1.4 decitex, 38 mm) and 65 mass% of a polyacrylic fiber staple (single fiber fineness: 1.0 decitex, 45 mm) were mixed by card mixing to obtain a spun yarn of 147 decitex.

The spun yarn thus obtained, a cation-dyeable polyester long fiber (90 decitex - 48 filaments), and a polyurethane-based elastic fiber (28 decitex - 2 filaments) were knitted into a greige fabric of a jersey structure using a single-knit knitting machine having a cylinder diameter of 76.2 cm and a gauge of 28 needles/2.54 cm. As the yarn length at the time of knitting, it was designed such that, after the following processing, the spun yarn would be measured 265.00 mm and the cation-dyeable polyester long fiber would be measured 250.00 mm, alternately repeated in the warp direction, and the polyurethane-based elastic fiber was knitted in parallel with each long fiber, respectively. The knitted fabric was 20 wt% of the viscose rayon, 38 wt% of the polyacrylic fiber, 34 wt% of the cation-dyeable polyester fiber, and 8 wt% of the polyurethane-based elastic fiber.

The greige fabric thus obtained was processed by steps of heat setting (190°C, 30 seconds) - scouring (70°C) - dyeing (115°C) - drying (130°C) - heat setting (130°C).

As a result of evaluating the yarn length, smoothness, and heat retaining property in the same manner as in Example 1 described above, it was confirmed that the heat retaining property was excellent, but the smoothness was poor.

**[Table 1]**

| | | Unit | Example 1 | Example 2 | Example 3 | Example 4 | Comparative Example 1 | Comparative Example 2 | Comparative Example 3 |
|---|---|---|---|---|---|---|---|---|---|
| Fiber 1 | Fiber type | | Acrylic/rayon spun yarn | Acrylic/rayon spun yarn | Acrylic/rayon spun yarn | Acrylic/rayon spun yarn | Polyester long fiber | Acrylic/cotton spun yarn | Acrylic/rayon spun yarn |
| | Total fineness D1 | Decitex | 125 | 125 | 98 | 98 | 110 | 147 | 147 |
| | Yarn length L1 | mm | 275.00 | 255.00 | 255.00 | 255.00 | 275.00 | 265.00 | 265.00 |
| Fiber 2 | Fiber type | | Polyester long fiber | Polyester long fiber | Polyester long fiber | Polyester long fiber | Polyester long fiber | Polyester long fiber | Polyester long fiber |
| | Total fineness D2 | Decitex | 84 | 84 | 56 | 56 | 84 | 33 | 90 |
| | Yarn length L2 | mm | 315.00 | 260.00 | 295.00 | 268.00 | 295.00 | 295.00 | 250.00 |
| D2/D1 | | | 0.67 | 0.67 | 0.57 | 0.57 | 0.76 | 0.22 | 0.61 |
| L2/L1 | | | 1.15 | 1.02 | 1.16 | 1.05 | 1.07 | 1.11 | 0.94 |
| Knitting | Structure | | Jersey | Jersey | Jersey | Jersey | Jersey | Jersey | Jersey |
| | GG | Gauge | 28GG | 28GG | 28GG | 28GG | 28GG | 28GG | 28GG |
| Smoothness | Tribomaster (Skin surface) | | 0.35 | 0.39 | 0.41 | 0.43 | 0.30 | 0.56 | 0.55 |
| Heat retaining property | CLO value | | 0.15 | 0.14 | 0.13 | 0.13 | 0.06 | 0.13 | 0.13 |

### DESCRIPTION OF REFERENCE SIGNS

- 1:: Fiber 1
- 2:: Fiber 2
- 3:: Elastic fiber
- 4:: Knitted fabric

## Claims

1. A knitted fabric having a single knit structure, wherein a course of a fiber 1 made of a spun yarn and a course of a fiber 2 made of a long fiber are alternately and repeatedly present in a warp direction, a ratio (D2/D1) of a total fineness D2 of the fiber 2 to a total fineness D1 of the fiber 1 is in a range of 0.50 to 0.90, and a ratio (L2/L1) of a yarn length L2 of the fiber 2 to a yarn length L1 of the fiber 1 per 100 wales is greater than 1.00.

2. The knitted fabric according to claim 1,
wherein the spun yarn contains a cellulose fiber and an acrylic fiber.

3. The knitted fabric according to claim 1,
wherein a total fineness D1 of the fiber 1 is 70 decitex to 150 decitex.

4. The knitted fabric according to claim 1,
wherein the long fiber is a cation-dyeable polyester long fiber.

5. The knitted fabric according to claim 1, wherein the total fineness D2 of the fiber 2 is 33 decitex to 135 decitex.

6. The knitted fabric according to claim 1 further comprising an elastic fiber.

7. The knitted fabric according to claim 1 further comprising a course of an elastic fiber.

8. The knitted fabric according to claim 1,
wherein the ratio (L2/L1) of the yarn length L2 of the fiber 2 to the yarn length L1 of the fiber 1 per 100 wales is in a range of 1.02 to 1.20.

9. A clothing comprising the knitted fabric according to any one of claims 1 to 8.

10. An undergarment or underwear made of the knitted fabric according to any one of claims 1 to 8.
